

## UNITED STATES PATENT OFFICE

1,943,000

## METHOD OF SIZING ARTIFICIAL FIBERS

Carroll Fred Chandler, Buffalo, N. Y., assignor,  
by mesne assignments, to Du Pont Rayon Com-  
pany, New York, N. Y., a corporation of Dela-  
ware

No Drawing. Application August 17, 1928  
Serial No. 300,374

14 Claims. (Cl. 91—68)

This invention relates to a method of sizing and more particularly to a method of sizing fibers, threads, or filaments having a cellulose derivative, such as an ether or ester, as a base.

5 Prior to this invention it has been the common practice to size artificial fibers having a cellulose derivative as a base with benzol or toluol solutions of sizing materials. These solutions are inflammable and, in addition thereto, 10 are quite expensive. Accordingly, it is desirable to use or employ an aqueous solution or emulsion for sizing. If fibers having a cellulose derivative as a base are sized in the same manner as cotton, artificial silk formed of regenerated cel- 15 lulose, or wool, it is found that very little sizing remains on the fibers. In fact, the quantity of sizing remaining on the fibers is insufficient to give them the desirable cohesion necessary in the weaving operation to which they are destined.

20 I have found that I can satisfactorily size fibers, threads or filaments having a cellulose derivative as a base with an aqueous sizing solution or emulsion by subjecting the fibers, threads or filaments to the combined action of a sizing material and 25 a swelling agent, the swelling agent serving to modify the said fibers, threads or filaments to permit satisfactory application and adhesion of the size thereto.

It is, therefore, an object of this invention to 30 provide a method of sizing fibers, threads or filaments having a cellulose derivative as a base with an aqueous solution or emulsion of a sizing material.

Another object of this invention is to provide 35 a method of sizing fibers, threads or filaments having as a base a cellulose derivative which comprises subjecting said fibers to the combined action of a swelling agent and a sizing material, the swelling agent serving to modify the said 40 fibers, threads or filaments to permit satisfactory application and adhesion of the size thereto.

Other objects will become apparent from the following description and appended claims.

To attain the above objects, skeins of artificial 45 silk are introduced or immersed in a solution or emulsion which contains a swelling agent for the cellulose derivative comprising the fibers, threads or filaments. After removing the excess of the 50 swelling agent, the swelled fibers, which retain an appreciable quantity of the solution in which they were submerged, are introduced into an aqueous sizing solution. Upon the removal of the fibers from the sizing bath, the treated fibers 55 are subjected to the usual finishing operations.

Instead of immersing the artificial silk in a solution or emulsion containing a swelling agent and then in the sizing solution, the artificial silk may be submerged, after a preliminary wetting with water, in a sizing bath containing the swell- 60 ing agent. After removal from the bath, the treated silk is finished in the usual manner.

If the artificial silk is in the form of warp threads, the process constituting this invention may be carried out in the usual slashing machines. 65

Various materials may be used as swelling agents. I have found that solutions of formaldehyde, acetone, acetic acid, formic acid, pyridine, phenol, salicylic acid, alkaline sulfocyanide, aniline, furfural and the like, emulsions or sus- 70 pensions of solvents of cellulose ethers or esters in water or in soap solutions produce satisfactory results.

If it is desired to increase the suppleness of the treated fibers, threads or filaments, materials, 75 such as soap, oil and the like, may be added to the sizing bath in any suitable quantity.

The sizing materials used are generally sub- 80 ject to mold or decay. Accordingly, by adding to the sizing bath a small quantity of any well-known disinfectant, such as boric acid, salicylic acid, phenol, and the like, the sizing solution may be preserved.

In order to more clearly explain the invention 85 the following examples are given. It is to be understood that these examples are merely illustrative and not limitative of the invention.

*Example I.*—One kilogram of cellulose acetate silk in skeins is immersed in an aqueous solution containing 20% of ammonium sulfocyanide for 90 one hour at approximately 25° to 30° C. Upon the removal of the skeins from this bath, they are rinsed, wrung and plunged into a bath containing 5% of gum arabic in which is emulsified 1% of cocoanut oil and .01% of boric acid. After 95 remaining in this bath for one hour, the skeins are wrung and dried in the usual manner.

*Example II.*—One kilogram of cellulose acetate silk, previously wetted in warm water, is im- 100 mersed in a solution containing 3% of gelatin, 0.25% of dextrin, 1% acetic acid, and 0.5% of sulphonated castor oil at 60° C. for approximately fifteen minutes. After wringing and drying, the cellulose acetate silk is found to be sized and is ready for weaving.

105 Since various modifications may be made in the above-described methods without departing from the nature of the invention, this invention is not limited to the specific details above set forth, except as defined in the following claims: 110

I claim:

- the class consisting of organic acid esters and ethers for the purpose of imparting thereto the cohesion and other characteristics desirable in the weaving thereof which comprises treating 5 said fibers, threads or filaments with a swelling agent and then with a sizing material, the swelling agent being of the class which consists of solutions of formaldehyde, acetone, acetic acid, formic acid, pyridine, phenol, salicylic acid, alkaline sulfocyanides, aniline, furfural, and emulsions or suspensions of solvents of cellulose ethers or esters in water or in soap solutions, said swelling agent serving to modify the material under treatment to permit satisfactory application and adhesion 80 of the size thereto.
12. A method of sizing artificial fibers, threads or filaments formed of a cellulose derivative of the class consisting of organic acid esters and ethers for the purpose of imparting thereto the cohesion and other characteristics desirable in the weaving thereof which comprises treating 10 said fibers, threads or filaments with a swelling agent and then with an aqueous solution containing a sizing material, the swelling agent being of the class which consists of solutions of formaldehyde, acetone, acetic acid, formic acid, pyridine, phenol, salicylic acid, alkaline sulfocyanides, aniline, furfural, and emulsions or suspensions of solvents of cellulose ethers or esters in water or in soap solutions, said swelling agent serving to modify the material under treatment to permit satisfactory application and adhesion of the size thereto. 15
13. A method of sizing artificial fibers, threads or filaments of cellulose acetate for the purpose of imparting thereto the cohesion and other characteristics desirable in the weaving thereof which comprises wetting the cellulose acetate material with water, immersing the wetted material in an aqueous solution containing gelatin and acetic acid, the acetic acid serving to modify the material under treatment to permit satisfactory application and adhesion of the size thereto, and drying the treated material. 20
14. A method of sizing artificial fibers, threads or filaments of cellulose acetate for the purpose of imparting thereto the cohesion and other characteristics desirable in the weaving thereof which comprises immersing the cellulose acetate material in a solution of ammonium sulfocyanide, removing the excess solution, and then immersing the material in a bath containing gum arabic. 25
- CARROLL FRED CHANDLER.
- 105
- 30
- 110
- 35
- 115
- 40
- 120
- 45
- 125
- 50
- 130
- 55
- 135
- 60
- 140
- 65
- 145
- 70
- 150
- 75